

## UNITED STATES PATENT OFFICE

2,145,996

## PROCESS OF PRODUCING A SCREENED WORK COPY OF AN ORIGINAL TO BE REPRODUCED

Wilhelm Schupp, Berlin, Germany, assignor of one-third to Paul A. Hennig, Hohokus, N. J., and one-third to Sydney Koppel, New York, N. Y.

No Drawing. Application June 11, 1937,  
Serial No. 147,675

4 Claims. (Cl. 95—5)

For reproducing black-white drawings, pictures etc. I have already proposed to use a positive or negative screened work copy of the original which copy is photographically transferred to a printing plate and which has been obtained by the aid of a screened negative and two continuous-tone negatives; the continuous-tone negatives serve as controlling means and compensate the flattening of the tint values due to the subdivision of the 5 screened negative into dots. In this process films are preferably used as sensitive carriers.

With regard to the three mentioned negatives the following conditions are to be considered.

The main or screened negative generally shall 10 not have well defined dots; the shadow dots (in the lightest portions of the negative) must be essentially larger than normally usual and the lights (the darkest portions of the negative) must be closed a little more than in case of screened 15 negatives hitherto used in the chemigraphy.

In the first continuous-tone negative the lights shall have only a delicate blackening; but within 20 the range of this delicate blackening the lights must have an extremely high contrast. This result is obtained by very short exposure of a 25 sensitive film, the index of gradation of which is very high (steep characteristic curve), and by utilizing a developer which automatically limits the blackening within the lightest portions.

The second continuous-tone negative is obtained from a sensitive film with a mean or less 30 high index of gradation, whereby the film is highly super-exposed and developed by a developer which also limits the blackening automatically.

From the three negatives thus obtained the 35 screened work copy may f. i. be produced in the following manner:

The three negatives and an unexposed sensitive film are superimposed so that in the direction of the printing light the films are lying behind each other in the sequence: first continuous-tone negative, screened negative, second continuous-tone negative, unexposed film. Thereafter the unexposed film is exposed through the 40 three negatives. The second continuous-tone negative is removed and the exposure repeated. The twice exposed film is then developed, fixed, toned down, until the highest lights are free from dots, and finally treated by means of an intensifier, so that the finest dots are sufficiently covered or blackened for the purpose of printing.

In the described method the quality of the reproduction essentially depends upon the corrective efficiency of the second continuous-tone negative, which controls the tone or tint values

of the screened negative within the shadows and which therefore is responsible for the production of well defined contours particularly between such portions and points of the reproduction which highly contrast with each other. In producing 5 this second continuous-tone negative it is therefore to be considered that besides limiting the blackening the creation of light courts or halos is carefully avoided.

I have found that the production of the second 10 negative is essentially simplified thereby that for its developing a developer is used which is composed of an aqueous solution of pyrocatechin and an aqueous solution of alkali carbonate (potash, sodium carbonate or mixtures thereof). As such 15 a developer not only avoids the creation of halos but also limits the blackening of the negative, it can also be utilized with great advantage for developing the first continuous-tone negative which controls the tone or tint values of the screened 20 negative within the lights.

I have f. i. obtained very satisfying results by using a developer composed of practically equal parts of a solution of about 5 g. pyrocatechin in 1000 ccm. water and of a solution of about 40 g. 25 potash in 1000 ccm. water. The quantity of pyrocatechin in the first solution and the quantity of potash in the second solution may be varied within certain limits. In any case, however, it is recommendable to maintain the relation 30 5:40 between pyrocatechin and potash.

It is to be considered that the developer is not stable; it decomposes after about 10 minutes. Therefore it is necessary that the developer is composed in the desired quantity just before it is 35 used.

What I claim is:

1. The process for producing a screened work copy of an original to be reproduced, which process comprises producing a main or screened negative of said original having the shadow dots thereon larger than normal and the lights closed more than normal, subjecting a sensitive film to a very short exposure to produce a first continuous-tone negative of said original, developing and fixing said first continuous-tone negative in a developer composed of an aqueous solution of pyrocatechin and an alkali carbonate, subjecting a sensitive film to high over-exposure to produce a second continuous-tone negative of said original, 40 developing and fixing said last mentioned negative, and superimposing the three negatives upon a sensitive film and exposing the negatives upon said sensitive film, 45

2. The process for producing a screened work

55

- copy of an original to be reproduced, which process comprises producing a main or screened negative of said original having the shadow dots thereon larger than normal and the lights closed more than normal, subjecting a sensitive film to a very short exposure to produce a first continuous-tone negative of said original, developing and fixing said negative in a developer composed of substantially equal parts of a solution of 5 g. pyrocatechin in 1000 ccm. of water and a solution of 40 g. potash in 1000 ccm. of water, subjecting a second sensitive film to high over-exposure to produce a second continuous-tone negative of said original, developing and fixing said last mentioned negative, and superimposing the three negatives upon a sensitive film and exposing the negatives upon said sensitive film.
3. The process for producing a screened work copy of an original to be reproduced, which process comprises preparing a main or screened negative having the shadow dots thereon larger than normal and the lights closed more than normal, subjecting a sensitive film to very short exposure to produce a first continuous-tone negative wherein the lights have a delicate blackening, developing and fixing said continuous-tone negative, preparing a second continuous-tone negative by over-exposing a sensitive film, developing and fixing the second continuous-tone negative in a developer composed of an aqueous solution of pyrocatechin and an alkali carbonate, superimposing the three negatives thus produced upon

an unexposed film with the screened negative intermediate the continuous-tone negatives, exposing the unexposed film through the superimposed negatives, removing the second continuous-tone negative and again exposing the superimposed negatives, developing, fixing and toning down the twice exposed film.

4. The process for producing a screened work copy of an original to be reproduced, which process comprises preparing a main or screened negative having the shadow dots thereon larger than normal and the lights closed more than normal, subjecting a sensitive film to very short exposure to produce a first continuous-tone negative wherein the lights have a delicate blackening, developing and fixing said continuous-tone negative, preparing a second continuous-tone negative by over-exposing a sensitive film, developing and fixing the second continuous-tone negative in a developer essentially comprising substantially equal parts of a solution of 5 g. pyrocatechin in 1000 ccm. of water and a solution of 40 g. potash in 1000 ccm. of water, superimposing the three negatives thus produced upon an unexposed film with the screened negative intermediate the continuous-tone negatives, exposing the unexposed film through the superimposed negatives, removing the second continuous-tone negative and again exposing the superimposed negatives, developing, fixing and toning down the twice exposed film.

WILHELM SCHUPP.